

No. 732,541.

PATENTED JUNE 30, 1903.

G. GERDOM.

GAS CHECK PAD FOR BREECH LOADING ORDNANCE.

APPLICATION FILED DEC. 27, 1902.

NO MODEL.

2 SHEETS—SHEET 1.

Fig. 1



Fig. 3



Fig. 2



Witnesses:

Raphael Fetter  
William W. Vogt.

Gregory Gerdom, Inventor

by J. D. Morrison Atty

No. 732,541.

PATENTED JUNE 30, 1903.

G. GERDOM.

GAS CHECK PAD FOR BREECH LOADING ORDNANCE.

APPLICATION FILED DEC. 27, 1902.

NO MODEL.

2 SHEETS—SHEET 2.

*Fig. 4*



*Fig. 5*



*Fig. 6*



Witnesses:

Raphael Ketter  
William M. Vogt

Gregory Gerdom, Inventor

by J. D. McCormick Atty

## UNITED STATES PATENT OFFICE.

GREGORY GERDOM, OF WATERVLIET, NEW YORK, ASSIGNOR TO ORDNANCE IMPROVEMENT COMPANY, A CORPORATION OF NEW YORK.

## GAS-CHECK PAD FOR BREECH-LOADING ORDNANCE.

SPECIFICATION forming part of Letters Patent No. 732,541, dated June 30, 1903.

Application filed December 27, 1902. Serial No. 136,770. (No model.)

*To all whom it may concern:*

Be it known that I, GREGORY GERDOM, of Watervliet, Albany county, New York, have invented a new and useful Gas-Check Pad for Breech-Loading Ordnance, of which the following is a specification.

My invention relates to improvements in gas-check pads for breech-loading ordnance, its object being to provide a pad which will be practically unaffected by extreme ranges of temperature and also which cannot be burned or otherwise injured by contact with the powder-gases.

To this end my invention consists in the improved plastic composition adapted to constitute the body of the pad and in the envelop therefor, both as hereinafter particularly described and claimed.

The type of gas-check for which my invention is adapted is known as the "De Bange," in which the pad is seated upon the forward end of the breech-block and a mushroom head bears upon the pad and has a stem extending through an axial opening in the pad and block.

In the service use of guns fitted with the above-described type of gas-check it has been found that the canvas envelop or covering for the pad is permanently injured or destroyed in case of slight leakage of gas which comes into contact with it. It is also found that the composition heretofore used in such pads by extreme cold is rendered too rigid for its designed function and that repeated firings of a gun will raise the temperature of the chamber and of the pad to such a degree that the composition is reduced to such soft condition that it fails to retain its normal shape and seriously interferes with the action of the breech-block. My improved composition, however, is practically unaffected by the extreme maximum and minimum temperatures to which it is subjected in service.

My improved pad envelop or covering, while perfectly flexible, so as to yield to pressures modifying the form of the pad, is wholly unaffected by the hot gases which may leak into contact with it. The composition for the core consists of the following ingredients com-

pounded in substantially the following proportions and manner: Take about four parts, by measure, of glycerin, with one part, by measure, of starch, mix and cook until reduced to a stiff paste and then add two parts, by measure, of tallow or linseed or other suitable oil and mix thoroughly while hot. The mass should then be allowed to stand for several days. This paste is then mixed with asbestos in about the following proportions—viz., twenty to thirty per cent of paste with eighty to seventy per cent of asbestos. This is thoroughly mixed and should be allowed to stand under pressure for several days, after which it is ready for molding into pads. The pad so molded is covered with the wire envelop in the manner hereinafter described.

In the accompanying drawings, forming part of this specification, Figure 1 represents a sectional side elevation of my improved pad before it is subjected to final pressure. Fig. 2 is a plan view of the pad complete, showing the interlocking and uniting edges of the covering. Fig. 3 is a side or edge elevation of the complete pad, a portion being broken away to show the embedding of the wires of the covering in the mass of the core under final pressure. Fig. 4 is an enlarged detail of a piece of the wire-netting used for the covering. Fig. 5 is a similar view of the same distorted, as when applied to the core; and Fig. 6 is a detail showing the interlocked edges of the netting as it is secured in place.

In the drawings, A represents the core of plastic material, and B its envelop of wire-netting. The general form of the core, as is well understood, is annular and properly shaped to fit its seat upon the end of the breech-block and the mushroom head which bears upon its opposite face. The composition hereinbefore described having been molded into the proper form is covered by the wire-netting B in the following manner: A piece of the netting, being distorted, as indicated in Fig. 5, in the direction of the plane of the pad, is folded around the outer periphery of the core and the meeting ends are interlocked by passing the wire ends 2 around the wire 3 of the opposite selvage edge and bending them

backward, as shown in Fig. 6. Similarly a piece of the netting is folded upon the inner periphery of the core and its ends united. The meeting and overlapping edges of the two pieces of fabric are then secured together, as shown in Figs. 1, 2, and 3, by laying an annular piece of asbestos or other non-conductor underneath the same and then uniting the wires by solder. After the pad has thus been completed it is subjected to heavy pressure, which forces the wires into the mass of the core or, conversely, the mass of the core out between the wires, so that the wires are completely embedded therein and a smooth surface is presented to the adjacent parts of the gun, as shown in Fig. 3. The envelop is free to yield to the pressures which modify the form of the pad, while retaining the contents, and is unaffected by a leakage of hot gases, which would burn and cut a combustible envelop. After the pad is finished it should be subjected for about one hour to a heat of about 300° Fahrenheit and after cooling should be given one or more coats of linseed-oil. After drying the pad should be returned to the press for final pressure and shaping.

I claim—

1. A gas-check pad, comprising a plastic core having a metallic cloth envelop. 30  
2. A gas-check pad comprising a plastic core and a wire-cloth envelop constructed substantially as specified.

3. A gas-check pad having a plastic core, and a wire-cloth envelop formed by folding 35 sections of cloth upon the core and uniting the overlapping edges with solder.

4. A gas-check pad comprising in combination a flexible envelop and a plastic core composed of asbestos, a suitable grease, glycerin and starch combined substantially in the proportions and manner specified. 40

5. A gas-check pad comprising in combination, a flexible wire-cloth envelop and a plastic core composed of asbestos, a suitable grease, glycerin and starch, constructed and combined substantially as specified. 45

Signed at New York city this 19th day of December, 1902.

GREGORY GERDOM.

Witnesses:

T. D. MERWIN,  
J. T. CRANE.